

# UNITED STATES PATENT OFFICE.

LUDWIG MACH, OF JENA, GERMANY.

## ALLOY OF ALUMINIUM.

SPECIFICATION forming part of Letters Patent No. 629,084, dated July 18, 1899.

Application filed February 25, 1899. Serial No. 706,848. (No specimens.)

*To all whom it may concern:*

Be it known that I, LUDWIG MACH, a subject of the Emperor of Austria-Hungary, residing at Jena, Empire of Germany, have invented a new and useful Alloy of Aluminium, of which the following is a specification.

This invention relates to a new and improved alloy of aluminium and magnesium. Heretofore, as is known to those familiar with the art, a most valuable quality of aluminium (its small specific gravity, 2.64) could not be made use of to the degree desired, because it was impossible neatly or finely to work the pure aluminium with cutting-tools. The faces worked show tears. The chips are composed of short splinters. The tools do not cut, but tear. Files are stopped up after a few touches and are rendered ineffective, so that the hand manipulating the file has more the feeling of ineffectually rubbing than that of shaping chips. In this respect the pure aluminium is inferior in these qualities even to pure copper, which, as is known, offers great difficulties to being worked. Hence for many years experiments have been directed to the improvement of the technological qualities of the aluminium by adding heavy metals—such as copper, nickel, &c.—naturally not without entailing a corresponding increase of specific weight. Although the chief advantage of the aluminium was thereby partly sacrificed, the improvement in result obtained did not answer expectations, it being impossible to turn to shape, to mill clean or satisfactory faces, or to cut sharp threads on pieces worked from these alloys of aluminium generally made use of. Further, it was found to be impossible to work them with good effect with fine files. This invention relates to an alloy of aluminium which allows of the working by cutting-tools in a perfect manner and yet diminishes the specific weight of the pure aluminium. It has been demonstrated by numerous experiments that magnesium, with its lighter specific gravity, (1.74,) alloyed with aluminium in certain proportions gives the latter those qualities with respect to its mechanical working and strength which the pure aluminium does not possess. From these experiments it resulted that in order to produce

the qualities mentioned as little as ten and no more than thirty parts, by weight, of magnesium may be added to one hundred parts of aluminium and that the proportion of ten to twenty-five parts of magnesium to one hundred parts of aluminium was the most advantageous.

If one hundred parts of aluminium are alloyed with ten parts of magnesium, the alloy has about the same mechanical qualities as rolled zinc. An alloy of one hundred parts of aluminium and fifteen parts magnesium corresponds to good foundry-brass, while an alloy of one hundred parts of aluminium and of twenty parts of magnesium gives the metal the character of a softer red brass or a brass wire hard drawn, and, finally, an alloy of twenty-five parts of magnesium and one hundred parts of aluminium represents the qualities of usual red brass.

This alloy may be founded in a thin fusible state. The pieces founded exhibit long curls of chips in turning or boring. Threads can be cut with sharp profiles, and the bore-holes are very fine and neat. The file makes a fine and regular "touch" or cuts without tearing or becoming stopped up. In filing the usual characteristic noise is heard. Heretofore only coarse or middling files could be employed, naturally at the cost of exactness. This alloy permits the use even of the finest files.

The pure aluminium can be cut with a knife like zinc, while the new alloy behaves like a piece of red brass beneath the edge of the knife. Yet these alloys, especially the softer alloys—one hundred parts aluminium and ten to fifteen parts magnesium—are very ductile and can be forged in a cold state, milled to plates, drawn to tubes and wire, and possess, therefore, the very valuable qualities of the pure aluminium.

The hardness and strength of the new alloy are so eminent that even axes, cock-pegs, &c., can be manufactured from it. The polish can be carried to brilliancy and is of an extraordinary resistance to the influence of the atmosphere. The color of the alloy is nearly silver white, differing from that of the pure aluminium, the color of which is somewhat unsightly. Besides these valuable workable qualities this new alloy of aluminium and magnesium possesses the invaluable superi-

ority that the specific weight not only is not increased, but is even reduced.

To this alloy of aluminium and magnesium heavy metals and alloys of them may be 5 added—such as copper, nickel, tungsten, and German silver; but except when intended for special purposes such an addition is not advisable, because, on the one hand, the specific weight of the alloy is increased and, on the 10 other hand, one can attain, even to the finest modifications, all the mechanical qualities by the aluminium-magnesium alloy, such as hardness and workable qualities. It has become evident that with such additions the 15 best results are obtained if only as much of the heavy metal is added to the alloy of aluminium and magnesium so long as the specific gravity of the pure aluminium be not exceeded.

20 An addition of heavy metals to alloys containing more than twenty parts of magnesium to one hundred parts of aluminium would be quite useless, because the unusual hardness and initial brittleness characteristic of this 25 addition would be disadvantageous to the working of the alloy. Experiments for alloying aluminium with magnesium had been begun at the time when aluminium was discovered. Wöhler (*Annalen der Chemie und Pharmacie*, 1866, Vol. 138, p. 253) fused these 30 two metals together in the proportions represented by  $Al_2Mg$ , forming an alloy with 69.2 per cent. of aluminium. The product was a tin-white mass, very brittle, igniting at red 35 heat, and burning with a white flame similar to magnesium alone. The alloy in the proportions  $Mg_2Al$ , containing thirty-six per cent. of aluminium, was malleable, but completely destroyed by leaving in water for a day without 40 any evolution of hydrogen. Wöhler stated his opinion with regard to these alloys as follows: "Both these mixtures appeared to contain a compound of definite composition, for when treated with a solution of 45 sal-ammoniac they disengaged hydrogen abundantly and deposited a brilliant, tin-white metallic powder. The solution contained magnesium chlorid, while the residue was rich in aluminium and appeared to produce 50 some aluminate of magnesium, which clouded the solution. The metallic residue was washed with water, again treated with sal-ammoniac solution, and then with solution of caustic soda until it no longer evolved 55 hydrogen. This residue was about one-third the total alloy and was insoluble in both the above reagents. It burned with brilliant sparks when thrown into a flame."

Parkinson, (*Journal für Practische Chemie*, 60 Vol. 101, p. 375,) after his experiments with magnesium alloys, says: "None of the mag-

nesium-aluminium alloys promises any practical utilization," and this at a time when Wöhler's experiments had long been known.

Muspratt (*Technische Chemie*, edition IV, 65 Vol. 5, p. 1026) comprises the result of the experiments made by White, Wanklyn and Chapman, Parkinson, and Mellor, so that all the alloys are very brittle and are more or less oxidized by the air and decomposed water to 70 a certain extent. Even to the present time this view has remained unchanged. This is seen by the circumstance that a modern author, such as Richards, who has thoroughly treated of aluminium has nothing else to 75 mention of the alloy of aluminium and magnesium but the results from the experiments of Wöhler, enumerating, as he does, the same compounds  $Al_2Mg$  (alloy with 69.2 per cent. 80  $Al$ ) and  $Mg_2Al$  (alloy with thirty-six per cent.  $Al$ ) and the same result as Wöhler, and this at a time when the practical importance was established beyond all doubt, which was not the case at the time of Wöhler, (cf. Richards, 85 *Aluminium*, edition II, p. 400.)

Once more, magnesium in connection with aluminium is mentioned in the English specification No. 21,575, of 1895. To obtain an alloy of aluminium possessing a greater tenacity than pure aluminium has, aluminium is mixed 90 with tungsten or magnesium as a copper-tin-tungsten alloy or copper-tin-magnesium alloy. Magnesium is contained in vanishing quantities (four per cent.) in this alloy, of which four to ten per cent. are added to the 95 aluminium, so as to leave still smaller quantities in the final alloy.

Having now described my invention, what I claim as new, and desire to protect by Letters Patent, is—

1. An aluminium-magnesium alloy herein described containing aluminium and magnesium in the proportions of one hundred parts of aluminium to between ten and thirty parts of magnesium substantially as and for the 105 purpose described.

2. An alloy comprising one hundred parts of aluminium, ten to thirty parts of magnesium, with copper, nickel, tungsten, and zinc, substantially as described.

3. An alloy including one hundred parts of aluminium, ten to thirty parts magnesium, and some heavier metal or metals, said alloy having a specific gravity no greater than aluminium.

In testimony that I claim the foregoing as my invention I have signed my name in presence of two subscribing witnesses.

LUDWIG MACII.

Witnesses:

ALVESTO S. HOGUE,  
WOLF PAULI.